

## 1

3,832,226

**METHOD FOR DRY ELECTROSTATIC COATING**  
Taizo Kondo and Keizo Inamura, Hiratsuka, Japan, assignors to Kansai Paint Company Limited, Amagasaki-shi, Hyogo-ken, Japan  
No Drawing. Original application May 13, 1969, Ser. No. 824,280, now abandoned. Divided and this application Apr. 27, 1971, Ser. No. 137,995  
Claims priority, application Japan, May 21, 1968, 43/34,472  
Int. Cl. B05b 4/02; B44d 1/92, 1/94  
U.S. Cl. 117—17 7 Claims

### ABSTRACT OF THE DISCLOSURE

A method for dry electrostatic coating of base metal surfaces to provide continuous, even, resin films free of pin-holes and cissings without the necessity of pre-heating the base metal by coating the surface of the base metal with a primer comprising a vehicle and an electroconductive particulate material having a particle size of not more than  $100\mu$ , such as aluminum powder, in an amount necessary to produce a dry film having a volume resistivity of  $10^9$  to  $10^{14}$  ohm-cm., and drying the film.

This application is a division of application Ser. No. 824,280 in the name of Taizo Kondo et al., filed May 13, 1969 (now abandoned).

This invention relates to an improved primer for electrostatic spraying of resin powder and a process for dry electrostatic coating of base metals with synthetic resin powder.

In recent years dry electrostatic coating method is widely being utilized for coating the surface of metal products with resins in various fields, since this process provides a number of important advantages as compared with liquid electrostatic coating methods. According to the principle of the conventional dry electrostatic coating methods a negative electrostatic charge is put on resin particles and the charged particles are sprayed to be brought near the base metal which is electrically grounded. Thus the particles are attracted to the base metal and deposited on it by Coulomb energy without losing their charge due to nonconductivity thereof. The deposited particles are then fused by heating in an oven to produce a continuous coating film.

According to the conventional methods, however, when the deposited particles are fused on the base metal they will lose Coulomb energy by the discharge due to rapid drop of electric resistance in proportion to the temperature, resulting in the particles easily falling off the surface of the base metal. The higher the melting point of the resin particles the more they are subject to this trend. When polyamide particles having a melting point of higher than  $150^\circ$  C. are directly deposited on a base metal by dry electrostatic coating method and fused on the base metal, for example, they discharge before they are heated to their melting point at which they coalesce with one another, leading to the deposited particles falling off. For this reason it has been considered difficult to produce a continuous polyamide coating film on a base metal by dry electrostatic coating methods. Even when polyvinyl chloride particles are deposited on a base metal they are liable to fall off in the melting step unless rapidly heated to their melting point.

## 2

To overcome this drawback and improve the properties of the resin coatings it is known in the art that primers may be applied to the surface of base metals prior to dry electrostatic coatings. If a primer is used, however, the electric resistance on the surface of the base metal coated therewith becomes so high that the base metal surface will easily have the same charge by the deposition of extremely small amounts of resin particles to cause the mutual repulsion of the particles on the surface, preventing deposition in a desired thickness. Thus the resultant molten film on the base metal is generally thin and finished with numerous pin holes or cissings and also with uneven thickness.

Various attempts have been made to solve these problems, but no successful methods have been proposed yet. In one known method, for example, a base metal is pre-heated to a temperature higher than the melting point of the resin particles deposited on the surface thereof so that the particles deposited are instantly melted on the surface to produce a continuous coating film. According to this method, however, a device for heating the base metal to such a high temperature is required, resulting in the loss of the inherent merit of electrostatic coating which requires no preheating of the base metal.

Another countermeasure is to preheat the base metal coated with a primer to about  $50$  to  $80^\circ$  C. so as to reduce the electric resistance of the particles to be deposited on the surface of the base metal by the subsequent electrostatic coating, and thereby mutual repulsion of the resin powder is minimized, making it possible to obtain the deposition of the particles in a desired thickness. According to this method, however, the release of the charge on the deposited particles reduces Coulomb energy, which results in poor adhesion of the particles to the metal base as easily falling off by relatively weak shock, such as conveyor line vibration. Further such method requires pre-heating device and complicated procedure for controlling the temperature of the heated base metal.

One object of the invention is accordingly to provide an improved primer for dry electrostatic coating which makes it possible to deposit resin particles in a desired thickness by dry electrostatic coating.

Another object of the invention is to provide improved primer for dry electrostatic coating which makes it possible to produce by dry electrostatic coating a continuous and even resin film which is firmly adhered to a base metal and has a desired thickness free from pin holes and cissings without preheating of the base metal.

A further object of the invention is to provide a method of electrostatic coating of a base metal with resin powder, whereby deposition of resin powder in a desired thickness may be secured.

A still further object of the invention is to provide a method of electrostatic coating of a base metal with resin powder, which makes it possible to produce a continuous and even resin film which is firmly adhered to a base metal and has a desired thickness free from pin holes and cissings, without any preheating of the base metal.

These and other objects of the invention will be apparent from the following description.

The primer composition for dry electrostatic coating of the invention comprises a vehicle and a particulate electro-conductive material dispersed in the vehicle; said electro-conductive material having a particle size of not more than  $100\mu$  and being contained in the amount ranging

from 10 to 60 weight parts, based on 100 weight parts of the binder resin in the vehicle and necessary for producing a dry film having a volume resistivity of  $10^9$  to  $10^{14}$  ohm-cm.

Throughout the specification and claims "volume resistivity" of the dry film of the present primer is defined from the following equation.

$$\text{Volume resistivity (ohm-cm.)} = \frac{A}{t} \times R_v$$

wherein  $t$  is thickness of dry film (cm.),  $A$  is area of main electrode ( $\text{cm.}^2$ ) and  $R_v$  is electric resistance measured in accordance with ASTM-257-61 in which mercury electrode is used and 100 v.-D.C. is applied using a test piece prepared by spraying a primer of the invention onto the surface of a degreased steel plate, 100 mm. x 100 mm. x 0.8 mm., to a thickness of  $20\mu$  in terms of dry film, followed by drying, and repeating this procedure to produce a dry film of  $500\mu$  thick on the steel plate.

The vehicle in the present primer is an organic solvent solution of a binder resin. Representatives of the binder resins are, for example, phenolic resins, vinyl chloride resins and epoxy resins, though other polymers may also be used for the purpose. These resins may be used singly or in mixture with one another or with acrylic resins. Although preferable resins may be selected in accordance with the kinds of the polymer powder to be deposited by electrostatic coating and the properties of the electrostatic coating film required to be improved, usually phenol resin, epoxy resin and polyvinyl chloride may preferably be used singly or in mixture with one another. The solvent used includes various organic solvents capable of dissolving the binder resin used, such as toluene, xylene, mineral spirits, methylethyl ketone, etc. The resin concentration of the solution may vary in accordance with the kinds of the resin used and the methods for coating, but it is preferable to be in the range of 15 to 50 weight percent, based on the combined weight of the resin and organic solvent. The most preferable concentration is 15 to 20 weight percent for polyvinyl chloride, 40 to 50 weight percent for phenol resin and 30 to 40 weight percent for epoxy resin.

The particulate electro-conductive materials used in the invention include powder of, for example, aluminium, silver, copper, bronze, carbon black, acetylene black, graphite, etc., most desirable being aluminium powder and graphite powder. The particle size of the materials is not larger than  $100\mu$ , preferably in the range of 0.01 to  $10\mu$ . The amount of the electro-conductive material is critical and it should be in the range of 10 to 60 weight parts, based on 100 weight parts of the binder resin in the vehicle. Further, by the addition of the electro-conductive materials within the above range the volume resistivity of the dry film defined before must be in  $10^9$  to  $10^{14}$  ohm-cm. Namely, the electro-conductive materials should be added in the amount necessary for producing the dry film of the primer having a volume resistivity of  $10^9$  to  $10^{14}$  ohm-cm. within the range of 10 to 60 weight parts, based on 100 weight parts of the binder resin. This amount is far high as compared with that of pigment used in the conventional primer. And unless the amount of the electro-conductive materials is within the above range, by dry electrostatic deposition there can not be obtained a continuous and even resin film which is firmly adhered to a base metal and has a desired thickness free from pin holes and cissings. For example, when the conductive materials are added in less than 10 weight parts, based on 100 weight parts of the binder resin, or if the volume resistivity of the dry film of the primer is higher than  $10^{14}$  ohm-cm., such primer results in the production of a thin film having undesired pin holes or cissings. And when the conductive materials are added in more than 60 weight parts, based on 100 weight parts of the binder resin, or if the volume resistivity of the dry film of the primer is lower than  $10^9$  ohm-cm., the resin particles deposited on the

primer film by electrostatic spraying easily fall off in melting step.

The preferable amount of the conductive materials is in the range of 20 to 50 weight parts, based on 100 weight parts of the binder resin, and the preferable volume resistivity of the dry film of the primer is in the range of  $10^{10}$  to  $10^{13}$  ohm-cm.

Though pigments or fillers may be added to the present primer, it is not desirable in the invention. When such additives are required it is preferable to add them in as small amount as possible, so as not to allow the undesired coagulation of the primer.

According to the invention, the surface of a base metal is coated with the present primer by various means, such as dipping, brushing, casting, rolling, spraying, electrostatic spraying, etc. and dried to obtain the dry film of the primer having a thickness of more than  $3\mu$ , preferably 10 to 100 $\mu$ .

Then resin powder is deposited on the primer film by the conventional dry electrostatic coating methods. As the primer film has a volume resistivity of  $10^9$  to  $10^{14}$  ohm-cm. the resin powder may be deposited to the desired thickness without mutual repulsion. The base metal is then heated in an oven to melt the deposited resin powder, whereby a continuous and even resin film having a desired thickness can be obtained free from undesired pin holes and cissings for the presence of the specific primer film of the invention.

The resin powder used in the electrostatic coating may include any one which has been used in the conventional dry electrostatic coating, for example, epoxy resins, olefin polymers, polyesters, polyamides, vinylchloride polymers, polycarbonates, cellulose derivatives, etc. These resins may be used singly or in mixture with one another. The resin powder may contain pigments, fillers and other additives, such as a plasticizer, curing agent, stabilizer, etc.

For better understanding of the invention Examples are given below, in which all parts and percentage are by weight.

#### EXAMPLE 1

100 parts of methylisobutylketone solution of resol type phenol resin containing 50 percent nonvolatile material, 100 parts of methylisobutylketone and 50 parts of cyclohexanone were mixed by stirring, to which was added non-leaving aluminium powder passing a 325 mesh screen in the proportions as shown in Table 1, and was further stirred homogeneously for 30 minutes, whereby a primer was obtained.

100 parts of polyamide particles and 5 parts of rutile-type titanium dioxide were mixed by a Henshell mixer at 3000 r.p.m. for 10 min., whereby the polyamide powder composition for dry electrostatic coating was prepared. The resultant product had the following characteristics:

Grain size \_\_\_\_\_ All passing 150 mesh.  
Softening point \_\_\_\_\_  $150^\circ$  C.  
Volume resistivity \_\_\_\_\_  $10^{11}$  ohm-cm.

A cold-rolled steel sheet, 200 mm. x 100 mm. x 0.8 mm. which was subjected to zinc phosphate parkerizing in accordance with Bonderite 144 standard process was coated by spraying with the primer of Table 1 below to dry film thickness of  $10\mu$ , and after being left at room temperature for 5 min. was heated in an air oven at  $180 \pm 5^\circ$  C. for 10 min. and then cooled. Then the test piece was coated with the above polyamide powder composition with "R-E-P gun" Trademark, electrostatic powder spray coating machine, of Ransburg (Japan, Ltd., Japan) at jet velocity of 210 g./min. for 10 sec. with uniform finish, and immediately heated in an air oven at  $200 \pm 5^\circ$  C. for 4 min. holding the coated surface vertical, and then cooled.

In the heating process the softening point of the polyamide powder composition,  $150^\circ$  C., was reached in 135 sec.

TABLE 1

| Experiment number                             | 1               | 2               | 3               | 4               | 5                | 6                 |
|-----------------------------------------------|-----------------|-----------------|-----------------|-----------------|------------------|-------------------|
| Composition of primer:                        |                 |                 |                 |                 |                  |                   |
| Phenol resin                                  | 100             | 100             | 100             | 100             | 100              | No primer used.   |
| Aluminum powder                               | 0               | 5               | 20              | 60              | 150              |                   |
| Volume resistivity (ohm-cm.)                  |                 |                 |                 |                 |                  |                   |
| $>10^8$                                       | $2 \times 10^6$ | $1 \times 10^4$ | $3 \times 10^2$ | $1 \times 10^8$ |                  |                   |
| Results of experiment:                        |                 |                 |                 |                 |                  |                   |
| Falling off during heating powder composition | None            | None            | None            | None            | Complete falling | Complete falling. |
| Average thickness of molten film ( $\mu$ )    | 130             | 140             | 270             | 260             |                  |                   |
| Uniformity of molten film                     | Cissing         | Cissing         | Good            | Good            |                  |                   |

As evident from the results of Table 1, when the volume resistivity of the dry film of the primer was less than  $10^8$  ohm-cm., or where no primer was used and the base metal was coated with polyamide powder composition direct by electrostatic spray coating, the polyamide powder composition deposited on the vertical surface started falling during the heating step and failed to form a film, whereas when it was more than  $10^{15}$  ohm-cm. the amount of deposited powder decreased throughout, and particularly the deposition of the powder composition

20 min. and then cooled. Then the sheet so primed was coated with the above polyvinyl chloride powder composition with "Stajet" (Trademark, electrostatic powder spray coating machine of Société Anonyme de Machines Electrostatiques, France) at jet velocity of 100 g./min. for about 10 sec., and immediately heated in an air oven at  $200 \pm 5^\circ$  C. for 15 min., holding the coated surface vertical. It required 240 sec. for the polyvinyl chloride powder composition to reach its softening point  $110^\circ$  C. during the heating process.

TABLE 2

| Experiment number                             | 7                    | 8                  | 9                  | 10                 | 11                 | 12              |
|-----------------------------------------------|----------------------|--------------------|--------------------|--------------------|--------------------|-----------------|
| Composition of primer:                        |                      |                    |                    |                    |                    |                 |
| Polyvinyl chloride                            | 80                   | 80                 | 80                 | 80                 | 80                 | No primer used. |
| Phenol resin                                  | 20                   | 20                 | 20                 | 20                 | 20                 |                 |
| Graphite powder                               | 0                    | 5                  | 20                 | 50                 | 100                |                 |
| Volume resistivity (ohm-cm.)                  |                      |                    |                    |                    |                    |                 |
| $>10^8$                                       | $5 \times 10^4$      | $6 \times 10^{13}$ | $2 \times 10^{10}$ | $1 \times 10^8$    |                    |                 |
| Results of experiment:                        |                      |                    |                    |                    |                    |                 |
| Falling off during heating powder composition | None                 | None               | None               | Partly falling off | Partly falling off |                 |
| Average thickness of molten film ( $\mu$ )    | 50                   | 90                 | 230                | 250                | 240                |                 |
| Uniformity of molten film                     | Pin holes throughout | Pin holes          | Good               | Good               |                    |                 |

was more difficult on the thick portion of the dry primer film, thus failing to form a uniform film and cissings were observed throughout the coated film. When the volume resistivity of the dry film of the primer was controlled to within  $10^8$  to  $10^{14}$  ohm-cm., excellent polyamide molten film free of the above faults was obtained.

#### EXAMPLE 2

400 parts of methylisobutylketone solution of copolymer of vinyl chloride, vinyl acetate and maleic anhydride, containing 20 percent non-volatile material and 40 parts of methylisobutylketone solution of resol type phenol resin containing 50 percent non-volatile material were mixed, to which was added graphite particles in the proportions as shown in Table 2 below and passed through 3-roll mill for three times to mix the components homogeneously, whereby primer composition was obtained.

The powder composition was prepared by mixing 100 parts of polyvinyl chloride particles, 30 parts of dioctylphthalate, 3 parts of organic tin compound and 6 parts of rutile type titanium dioxide, and stirring the mixture with a Henshell mixer at 3000 r.p.m. for 30 min. The resultant polyvinyl chloride powder composition had the following characteristics:

Grain size All passing 100 mesh.  
Softening point  $110^\circ$  C.  
Volume resistivity  $10^{10}$  ohm-cm.

35 The primer of Example 1 was coated on a cold-rolled steel plate in the manner same as in Example 1 except varying the thickness of the dry film of the primer as shown in Table 3 below, and the polyamide powder composition of Example 1 was applied thereto in the same manner as in Example 1 with the results shown in 40 Table 3.

TABLE 3

| Experiment number                                | 13          | 14   | 15   |
|--------------------------------------------------|-------------|------|------|
| Thickness of primer film ( $\mu$ )               | 1           | 3    | 10   |
| Results of experiment:                           |             |      |      |
| Falling off during heating of powder composition | Falling off | None | None |
| Average thickness of molten film ( $\mu$ )       | 250         | 230  |      |
| Uniformity of molten film                        | Good        | Good |      |

#### EXAMPLE 4

55 The primer of Example 1 was coated on a cold-rolled steel plate in the same manner as in Example 1 except varying the thickness of the dry primer film as shown in Table 4 below, and the polyvinyl chloride powder composition of Example 2 was applied thereto in the same manner as in Example 2 with the results shown in Table 4 below.

TABLE 4

| Experiment number                               | 16              | 17                   | 18                   | 19              | 20              | 21              |
|-------------------------------------------------|-----------------|----------------------|----------------------|-----------------|-----------------|-----------------|
| Composition of primer:                          |                 |                      |                      |                 |                 |                 |
| Phenol resin (parts)                            | 100             | 100                  | 100                  | 100             | 100             | 100             |
| Aluminum powder (parts)                         | 5               | 5                    | 5                    | 20              | 20              | 20              |
| Volume resistivity of dry primer film (ohm-cm.) | $2 \times 10^4$ | $2 \times 10^4$      | $2 \times 10^4$      | $1 \times 10^4$ | $1 \times 10^4$ | $1 \times 10^4$ |
| Thickness of dry primer film ( $\mu$ )          | 7               | 25                   | 48                   | 4               | 28              | 42              |
| Results of experiment:                          |                 |                      |                      |                 |                 |                 |
| Falling off during heating of deposited powder  | None            | None                 | None                 | None            | None            | None            |
| Average thickness of molten film ( $\mu$ )      | 150             | 90                   | Almost no deposition | 220             | 220             | 200             |
| Uniformity of molten film                       | Pin holes       | Pin holes throughout | Good                 | Good            | Good            | Good            |

A cold-rolled steel sheet, 200 mm. x 100 mm. x 5 mm. which was subjected to zinc phosphate parkerizing according to Bonderite 144 standard process was coated with the primer at Table 2 diluted with methylisobutylketone to obtain dry film about  $5\mu$  thick by spraying method, and after being left at room temperature for 5 min. was heated in a hot-air drier at  $180 \pm 5^\circ$  C. for

70 75 What we claim is:

1. A method for dry electrostatic coating a base metal with resin powder which comprises the steps of:  
(1) coating the surface of the base metal with the primer of a vehicle and a particulate electroconductive material dispersed in the vehicle, said vehicle being an organic solvent solution of at least one binder

resin selected from the group consisting of phenolic resin, epoxy resin and vinyl chloride resin, said solution having a concentration of 15 to 50 weight percent based on the combined weight of the resin and organic solvent, said electroconductive material being one species selected from aluminium powder, silver powder, copper powder, bronze powder, acetylene, black powder and graphite powder, and having a particle size of not more than  $100\mu$ , and being contained in the amount ranging from 10 to 60 weight parts based on 100 weight parts of the binder resin in the vehicle, and being necessary for producing a dry film having a volume resistivity of  $10^9$  to  $10^{14}$  ohm-cm.,

(2) heating the primer film at  $180 \pm 5^\circ$  C. for 10 to 20 minutes to obtain the dry film having a thickness of at least  $3\mu$  and a volume resistivity of  $10^9$  to  $10^{14}$  ohm-cm.,

(3) electrostatically coating the resin powder on the primer film thus obtained, and then,

(4) heating the resin powder to melt and form a continuous film on the primer film.

2. The method according to claim 1, in which said particulate electro-conductive material has a particle size ranging from 0.01 to  $10\mu$ .

3. The method according to claim 1, in which said particulate electro-conductive material is contained in the range of 20 to 50 weight parts, based on 100 weight parts of the binder resin.

4. The method according to claim 1, in which said particulate electro-conductive material is contained in the amount necessary for producing a dry film having a volume resistivity of  $10^{10}$  to  $10^{13}$  ohm-cm.

5. The method according to claim 1, in which said primer is coated on the base metal in a dry film thickness of 10 to  $100\mu$ .

6. The method according to claim 1 in which said resin powder is at least one species selected from epoxy resins, olefin polymer, polyesters, polyamides, vinylchloride polymers, polycarbonates or cellulose derivatives.

7. The method according to claim 6 in which said resin powder contains pigments and fillers.

#### References Cited

##### UNITED STATES PATENTS

|    |           |         |                |       |         |
|----|-----------|---------|----------------|-------|---------|
| 10 | 3,497,376 | 2/1970  | Wieser         | ----- | 117-17  |
|    | 3,672,927 | 6/1972  | Spiller et al. | ----- | 117-17  |
|    | 3,502,492 | 3/1970  | Spiller        | ----- | 117-17  |
|    | 3,327,685 | 6/1967  | Heyl et al.    | ----- | 117-33  |
|    | 3,056,750 | 10/1962 | Pass           | ----- | 252-512 |
|    | 3,083,169 | 3/1963  | Weda           | ----- | 252-512 |
|    | 3,278,455 | 10/1966 | Feather        | ----- | 252-512 |
|    | 3,328,317 | 6/1967  | McKeand et al. | ----- | 252-511 |
|    | 3,332,867 | 7/1967  | Miller et al.  | ----- | 252-512 |
|    | 3,496,911 | 2/1970  | Chmelar        | ----- | 117-17  |
|    | 3,551,178 | 12/1970 | Chmelar        | ----- | 117-17  |
|    | 3,030,237 | 4/1962  | Price          | ----- | 117-227 |
|    | 3,412,043 | 11/1968 | Gilliland      | ----- | 117-227 |
|    | 3,577,274 | 5/1971  | Taylor et al.  | ----- | 117-227 |
|    | 3,639,121 | 2/1972  | York           | ----- | 117-226 |

#### OTHER REFERENCES

Delmonte, *Metal-Tilled Plastics*, Reinhold, N.Y. (1961), pp. 174-183.

Handbook of Chemistry & Physics, pg. 2627, 44th edition.

MICHAEL SOFOCLEOUS, Primary Examiner

U.S. Cl. X.R.

35 117-226, 227